

1

2,693,432

## GLAZING BATTING MATERIALS

Fred Fortress, Summit, N. J., assignor to Celanese Corporation of America, New York, N. Y., a corporation of Delaware

No Drawing. Application January 25, 1951,  
Serial No. 207,835

9 Claims. (Cl. 154—137)

This invention relates to the glazing of batting materials and relates more particularly to an improved process for the glazing of batting materials formed from organic thermoplastic staple fibers.

Batting materials formed from organic thermoplastic staple fibers have found extensive use in a number of fields. Batting materials having a relatively substantial thickness are employed as structural insulation. In a much thinner form, the batting materials serve as linings and interlinings for garments of various types. One difficulty experienced in the application of said batting materials is that they do not have a sufficiently coherent structure to prevent their shredding and separating, particularly during the handling involved in using the same.

It has previously been proposed to reinforce the batting materials by stitching, but the stitching operation greatly increased the cost of said batting materials and thereby limited their field of use. Another expedient suggested for reinforcing the batting materials was to subject the same to some form of heat treatment to cause the organic thermoplastic staple fibers to coalesce with adjoining fibers, rendering the structure of the batting materials more coherent. To avoid a serious loss in the insulating properties of the batting materials, efforts were made to control the heat treatment so as to cause the fibers at the surface only of the batting materials to coalesce with adjoining fibers, which treatment is called "glazing." However, when heat alone was employed to glaze the batting materials, the high temperature required rendered it difficult to prevent the coalescence of staple fibers throughout the entire thickness of the batting materials and/or the degradation of the staple fibers at the surface of said materials. If, on the other hand, the staple fibers were treated with a plasticizer to permit said batting materials to be glazed at a lower temperature, the major portion of the plasticizer, which was in the body of the batting materials, was wasted.

It is an important object of this invention to provide a process for the glazing of batting materials formed from organic thermoplastic staple fibers which will be free from the foregoing and other disadvantages.

A further object of this invention is to provide an improved process for the glazing of batting materials formed from organic thermoplastic staple fibers to produce a coherent structure, which may be carried out at a reduced temperature and which will produce a uniform coalescence of the staple fibers at the surface only of the batting materials without wasting any materials.

Other objects of this invention will be apparent from the following detailed description and claims.

I have now discovered that batting materials formed from organic thermoplastic staple fibers may be glazed uniformly at a reduced temperature to provide a strong, flexible, fused, porous surface and a strong coherent structure, if there is applied to the surface of the batting materials an aqueous solution or dispersion, hereinafter referred to generally as an aqueous solution, of a softening agent for the organic thermoplastic staple fibers having a boiling point above about 125° C., and the so-treated batting materials are then immediately subjected to the desired heat treatment as, for example, by subjecting the same to the action of a heated surface. The batting materials treated in accordance with this process exhibit a uniform coalescence of the staple fibers at the surface only so that they retain the major portion of their insulating properties. In addition, the structure of the batting materials is sufficiently coherent to prevent their shred-

2

ding and separating during the handling normally encountered in using the same.

For the preparation of the batting materials there may be employed any standard carding machines having a batting attachment in combination therewith, as is well known in the art. The organic thermoplastic staple fibers from which the batting materials are formed preferably comprise an organic derivative of cellulose as, for example, cellulose esters such as cellulose acetate, cellulose propionate, cellulose butyrate, cellulose acetate propionate and cellulose acetate butyrate, and cellulose ethers such as ethyl cellulose and benzyl cellulose. The staple fibers may also be formed from organic thermoplastic materials as, for example, polyamides, polyurethanes, polytriazoles and vinyl polymers and copolymers. There may be mixed with the organic thermoplastic staple fibers staple fibers of materials that are not thermoplastic as, for example, cotton, silk, wool, regenerated cellulose, jute, hemp and asbestos fibers. In forming the batting materials, the staple fibers are interlaced and matted together so that they exhibit some degree of coherence even before the glazing operation.

In carrying out the process of this invention, there is applied to the surface of the batting materials an aqueous solution of a softening agent for the organic thermoplastic material having a boiling point above about 125° C. The softening agent may be a solvent, swelling agent or plasticizer for the organic thermoplastic material and may be a high boiling liquid or solid. Suitable softening agents include, for example, glycerol diacetate, glycol diacetate, dimethoxy tetraethylene glycol, diethylene glycol monoethyl ether, acetylacetone, triethylphosphate, ethyl lactate, diethylene glycol, urea, acetamide, potassium thiocyanate and boric acid. The softening agent must, as pointed out above, have a boiling point above about 125° C. since it has been found that softening agents having a lower boiling point are largely flashed off and therefore do not efficiently effect the glazing of the batting materials to provide a strong, flexible, fused, porous surface. The aqueous solution of the softening agent advantageously has a concentration of between about 5 and 20% by weight and is applied to the batting materials in amount sufficient to deposit from about 0.025 to 0.4 ounce of softening agent for each square yard of surface of the batting materials being treated. The aqueous solution of the softening agent may be applied to one or both surfaces of the batting materials and may be readily sprayed onto said surfaces through the use of suitable nozzles. Through the application of the softening agents in the form of aqueous solutions, it is possible to apply solid as well as liquid softening agents and to distribute the softening agents uniformly over the surface of the batting materials despite the small quantities of said agents that are employed. Certain of the softening agents, such as urea, boric acid and triethylphosphate have fire-retardant properties and will provide a fire-retardant surface on the batting materials in addition to assisting the glazing operation.

The batting materials are subjected to the action of a heated surface immediately after the aqueous solution of the softening agent is applied to the surface of said batting materials, and before said solution has an opportunity to diffuse into the interior of said batting materials. In this way, the coalescence of the organic thermoplastic staple fibers in the interior of said batting materials is substantially avoided. The temperature of the heated surface is advantageously maintained between 120 and 150° C. when glazing batting materials formed from staple fibers having a basis of cellulose acetate, and said heated surface is applied to the batting materials for a period of time sufficient to bring the temperature at the surface of the batting materials to between about 110 and 140° C. Suitable apparatus that may be employed in applying a heated surface to the batting material include presses, calender rolls and the like.

The following examples are given to illustrate this invention further.

### Example I

A batting material formed from interlaced and matted cellulose acetate staple fibers and having a thickness of

between  $\frac{3}{4}$  and  $\frac{1}{2}$  inches is sprayed on one surface with a 10% by weight aqueous solution of glycol diacetate in an amount sufficient to deposit 0.2 ounce of the glycol diacetate on each square yard of the batting surface. Immediately after the spraying is completed, the batting is contacted for 3 seconds and under a pressure of 2 pounds per square inch with a heating element maintained at 132-138° C. Upon removing the heating element, it is found that the batting is glazed uniformly at its surface only, exhibits a strong, flexible, fused, porous surface and has a firm coherent structure.

*Example II*

The process described in Example I is repeated employing a 10% by weight of a warm solution of boric acid and depositing 0.2 ounce of boric acid per square yard of batting surface. The batting is glazed uniformly at its surface only, exhibits a strong flexible, fused, porous surface and has a firm coherent structure.

*Example III*

The process described in Example I is repeated employing a 10% by weight solution of urea and depositing 0.2 ounce of urea per square yard of batting surface. The batting is glazed uniformly at its surface only, exhibits a strong, flexible, fused, porous surface and has a firm coherent structure.

*Example IV*

The process described in Example I is repeated employing a 10% by weight solution of acetamide and depositing 0.2 ounce of acetamide per square yard of batting surface. The batting is glazed uniformly at its surface only, exhibits a strong, flexible, fused, porous surface and has a firm coherent structure.

It is to be understood that the foregoing detailed description is given merely by way of illustration and that many variations may be made therein without departing from the spirit of my invention.

Having described my invention, what I desire to secure by Letters Patent is:

1. Process for the glazing of batting materials formed from organic derivative of cellulose staple fibers interlaced and matted together, which comprises applying to the surface of the batting materials an aqueous solution of a normally solid softening agent for the organic derivative of cellulose material, in an amount sufficient to deposit from about 0.025 to 0.4 ounce of softening agent per square yard of the surface of the batting materials, and subjecting the batting materials to the action of a heated surface whereby the organic derivative of cellulose staple fibers are coalesced at the surface only of the batting materials.

2. Process in accordance with claim 1 wherein the normally solid softening agent for the organic derivative of cellulose material is urea.

3. Process in accordance with claim 1 wherein the normally solid softening agent for the organic derivative of cellulose material is boric acid.

4. Process in accordance with claim 1 wherein the normally solid softening agent for the organic derivative of cellulose material is acetamide.

5. Process for the glazing of batting materials formed from cellulose acetate staple fibers interlaced and matted together, which comprises applying to the surface of the batting materials an aqueous solution of a normally solid softening agent for the cellulose acetate material, in an amount sufficient to deposit from about 0.025 to 0.4 ounce of softening agent per square yard of the surface of the batting materials, and subjecting the batting materials to the action of a heated surface whereby the cellulose acetate staple fibers are coalesced at the surface of the batting materials.

6. Process for the glazing of batting materials formed from cellulose acetate staple fibers interlaced and matted together, which comprises applying to the surface of the batting materials a 5 to 20% by weight aqueous solution of a normally solid softening agent for cellulose acetate material in an amount sufficient to deposit from about 0.025 to 0.4 ounce of softening agent per square yard of the surface of the batting materials, and, without permitting the aqueous solution to diffuse into the interior of the batting materials, subjecting the batting materials to the action of a heated surface having a temperature of between about 120 and 150° C. whereby the cellulose acetate staple fibers are coalesced at the surface only of the batting materials.

7. Process in accordance with claim 5 wherein the normally solid softening agent for the cellulose acetate material is urea.

8. Process in accordance with claim 5 wherein the normally solid softening agent for the cellulose acetate material is boric acid.

9. Process in accordance with claim 5 wherein the normally solid softening agent for the cellulose acetate material is acetamide.

References Cited in the file of this patent

UNITED STATES PATENTS

|    | Number    | Name      | Date          |
|----|-----------|-----------|---------------|
| 45 | 2,126,754 | Dreyfus   | Aug. 16, 1938 |
|    | 2,126,823 | Schneider | Aug. 16, 1938 |
|    | 2,497,117 | Dreyfus   | Feb. 14, 1950 |

FOREIGN PATENTS

|    | Number  | Country       | Date          |
|----|---------|---------------|---------------|
| 50 | 387,876 | Great Britain | Feb. 16, 1933 |
|    | 399,811 | Great Britain | Oct. 9, 1933  |
|    | 582,006 | Great Britain | Nov. 1, 1946  |